

## UNITED STATES PATENT OFFICE.

ROBERT W. R. MACKENZIE, OF EARSHOLL, FIFE, ERNEST H. ROBINSON, OF PERTH, MORRIS FORT, OF ALMONDBANK, AND JAMES DAVID LUMSDEN, DECEASED, LATE OF ALMONDBANK, SCOTLAND, BY SUSAN A. R. F. LUMSDEN, OF HUNTINGTOWERFIELD, ALMONDBANK, SCOTLAND; ROBERT W. R. MACKENZIE, OF EARSHOLL, FIFE, SCOTLAND; JOHN G. MILLER, OF PERTH, SCOTLAND; ROBERT O. LUMSDEN, OF ALMONDBANK, SCOTLAND; AND ALEXANDER P. MELVILLE, OF EDINBURGH, SCOTLAND, EXECUTORS OF SAID JAMES DAVID LUMSDEN.

## BEETLING AND TREATMENT OF FABRICS.

No Drawing.

Application filed December 28, 1920. Serial No. 433,745.

(GRANTED UNDER THE PROVISIONS OF THE ACT OF MARCH 3, 1921, 41 STAT. L., 1313.)

*To all whom it may concern:*

Be it known that ROBERT WALKER RANNIE MACKENZIE and ERNEST H. ROBINSON, subjects of the King of Great Britain and Ireland and the Isle of Man, residing, respectively, in Earlsholl, Fife, Scotland, and Stormontfield, Perth, Scotland, MORRIS FORT, a subject of the King of Great Britain and Ireland and the Isle of Man, residing in 5 Cromwell Cottage, Almondbank, Perthshire, Scotland, did, in connection with JAMES DAVID LUMSDEN, formerly a subject of the King of Great Britain and Ireland and the Isle of Man, residing in Huntingtowerfield, 10 Almondbank, Perthshire, Scotland, but now deceased, during his lifetime, invent Improvements in and Relating to the Beetling and Treatment of Fabrics (for which we have filed applications in England, Patent 15 No. 137,968, filed April 5, 1919; France, application No. 130,264, filed July 8, 1920; Belgium, application No. 231,193, filed July 9, 1920; Germany, application No. L. 50,923, filed July 6, 1920; Czechoslovakia, Patent 20 No. 5,591, filed July 9, 1920), of which the following is a specification.

Our invention relates to a process of treating fabrics, having particular relation to beetling processes.

30 An important object of our invention is

to provide a method of beetling bleached or unbleached fabrics which are composed of vegetable fibers.

Another object of our invention is to provide a treatment for fabrics which permits 35 the beetling of certain fabrics heretofore considered incapable of satisfactory beetling and which results in a fabric having greatly improved characteristics, all as will appear more fully hereinafter.

40 Other objects and applications of our invention, as well as the details of the process involved therein, will be apparent from the following description of the nature, the mode of operation, and the particular advantages 45 of our invention.

We have discovered that the effectiveness of a beetling treatment, when applied to fabrics composed of cotton, linen, or other vegetable fibers, is largely dependent upon 50 the moisture content and distribution of the same and also upon the presence of small amounts of oily, fatty, waxy, soapy, or resinous matter, which may be naturally included in the fabric or applied during the 55 treatment thereof. For example, one of two similarly bleached cotton fabrics, which failed to respond satisfactorily to a beetling treatment, was found to contain 0.19% of waxy and fatty matter; whereas the other 60

piece, which responded well to the beetling treatment, contained only 0.05% of waxy and fatty material. However, after the fabrics were treated, according to our invention, with a suitable solvent, each responded equally well to the beetling treatment and the maximum effect as to firmness and closure of the fabric interstices obtained.

Our invention, therefore, comprises a process, wherein the material under treatment is first treated to remove the oil, fat, wax and resin content thereof, and thereafter subjected to a beetling operation.

In the application of our invention to fabrics containing saponifiable oils and waxes, say of the mineral type, which have recently entered considerably into the composition of sizes applied to linen and cotton yarns before weaving, the solvent treatment is usually carried out on the dry fabric as it is received from the loom or after singeing or at any stage prior to the beetling operation. When the oils and waxes have been removed, the beetling operation may be performed after damping, even before the fabric is dry.

Our invention is also applicable to brown, grey, green, half bleached linen, and cotton goods which may be rendered as susceptible to beetling as the correspondingly perfectly bleached cloth without resort to the ordinary scouring and bleaching methods. Similar results are obtained with unbleached, half bleached, and bleached fabrics containing various natural and extraneous impurities associated with cellulose, other than oil, fat, wax and resin. The process constituting our invention, as applied to fabrics of the types just specified, comprises a dry cleaning treatment or an extraction treatment with a volatile solvent, such, for example, as benzene, benzine, naphtha, alcohol, ether, or any other known solvent or solvent mixture capable of dissolving oils, fats, waxes, and resins, which may be present in a free state or associated with mineral or organic matter. The solvent treatment may be carried out, if desired, in the presence of heat or under modified pressure at any stage in the treatment of the fabric. Where it is necessary for the goods to be mercerized, scoured, dyed, or bleached, the solvent treatment is preferably carried out before the operation just mentioned, to insure good beetling and to permit of the more effective use of the scouring and bleaching process for the control of the purity or whiteness of the treated fabric.

Our invention is particularly useful in the beetle-finishing of colored goods, as, for instance, linen and cotton goods containing dyed or colored threads, which are sometimes required to withstand bleaching before

beetling. By reason of the necessity for a milder boiling and scouring treatment for goods of the class herein specified than can be given to ordinary plain goods, in order that the colors shall not be impaired, an inferior white often obtains, and the presence of the fatty or waxy matter results in poor beetling. The undesirable results just mentioned are overcome by our invention and a mild scouring and bleaching treatment only are necessary after the solvent treatment to give the goods a suitable white color. Moreover the dyed threads are better preserved as to color and fully protected against staining or bleeding.

In the application of our invention to fabrics, which are first dyed and subsequently beetled, the solvent treatment is carried out while the goods are dry before the scouring and dyeing of the same. If desired, mild scouring treatments may be given subsequent to the solvent treatment to effect such cleansing as may be necessary. Where fabrics are required to be scoured and bleached but not dyed, ordinary scouring treatment with lime or alkalis may be given to effect a further cleansing action, and it has been found that such scouring treatment is more effective subsequent to the solvent treatment embodied in our invention.

Our invention is also applicable to such materials as mercerized, natural, white and colored or dyed linen and cotton damasks, dress goods, upholstery cloths and sheetings, where a good beetled finish is absolutely essential. The treatment for goods of the class just specified may be practiced at any stage of procedure after weaving, as a simple operation or in conjunction with scouring, bleaching, malting, dyeing, mercerizing, finishing or other such known operations as may be required to be performed in order to obtain certain other desired properties of whiteness, purity, color, lustre or finish. Subsequent to the solvent treatment, the beetling may be performed rapidly and perfectly at any desired stage on unbleached, mercerized, dyed, colored, or bleached cloth.

Although we have not described all the possible modifications and applications of our invention which could be conceived by one skilled in the art, it is apparent that various changes and modifications can be made therein without departing from the spirit of our invention, and we desire, therefore, that only such limitations shall be imposed thereon, as are indicated in the appended claims or as are demanded by the prior art.

What we claim is:

1. The process of beetling piece fabrics composed of vegetable fibres, which comprises treating the fabrics to remove the oil,

fat, wax and resin content, and thereafter subjecting the fabrics to a beetling operation.

2. The process of beetling piece fabrics composed of vegetable fibres, which comprises treating the fabrics with volatile solvents to remove the oil, fat, wax and resin content, and thereafter subjecting the fabrics to a beetling operation.
- 10 3. The process of beetling unbleached or partially bleached piece fabrics composed of vegetable fibres, which comprises treating the fabrics to remove the oil, fat, wax and resin content, and thereafter subjecting the fabrics to a beetling operation.

In witness whereof, the said ROBERT WALKER RANNIE MACKENZIE, ERNEST ROBINSON, MORRIS FORT, and SUSAN ANN RANKINE FORTUNE LUMSDEN, ROBERT WALKER RANNIE MACKENZIE, JOHN GARDNER MILLER, ROBERT OSWALD LUMSDEN and ALEXANDER PATRICK MELVILLE, executors of the estate of James David Lumsden, deceased, have hereunto set their hands.

R. W. R. MACKENZIE,  
ERNEST H. ROBINSON,  
MORRIS FORT,

*Inventors,*  
and

S. A. R. F. LUMSDEN,  
R. W. R. MACKENZIE,  
J. G. MILLER,  
R. O. LUMSDEN,  
ALEX. P. MELVILLE,

*Executors of the estate of James David Lumsden, deceased.*

Witnesses as to the signatures of R. W. R. Mackenzie, Ernest Robinson, Morris Fort, S. A. R. F. Lumsden, R. W. R. Mackenzie, J. G. Miller, and R. O. Lumsden:

D. A. COATES,  
PETER PATON.

Witnesses as to the signature of Alex P. Melville:

ALASTAN H. CREVAR,  
JOHN H. M. SOMERVILLE.